

July 19, 1960

L. P. JAHNKE ET AL

2,945,758

NICKEL BASE ALLOYS

Filed Feb. 17, 1958



Fig 1



Fig 2

INVENTORS  
LOUIS P. JAHNKE  
MARVIN A. POHLMAN  
BY  
*Lee H. Sacks*

ATTORNEY—

# United States Patent Office

2,945,758

Patented July 19, 1960

三

2,945.758

## NICKEL BASE ALLOYS

**Louis Prehn Jahnke, Cincinnati, Ohio, and Marvin A. Pohlman, Muskegon, Mich., assignors to General Electric Company, a corporation of New York**

Filed Feb. 17, 1958, Ser. No. 715,565

**6 Claims. (Cl. 75—171)**

This invention relates to nickel base alloys. More particularly, it relates to nickel base alloys which include a critical range of aluminum and titanium to produce unusual high strength properties at both low and high temperatures.

In order to advance the technology of operations such as that of high temperature operating turbines in which both low and high temperatures as well as high stresses are encountered, it has been necessary to develop materials having unusual strength properties at operating temperatures. Nickel base alloys have been attractive for such uses but have had, heretofore, strength limitations which have precluded their use for high stress applications especially at high temperatures.

Attempts have been made to strengthen nickel base alloys using combinations of molybdenum, titanium and aluminum as ingredients of the alloy and still maintain reasonable workability and ductility. Relatively broad ranges of these elements have been reported in nickel base alloys, but it has never before been recognized that a certain critical and narrow range of proportions of titanium and aluminum will produce certain unexpected properties. It has likewise never been recognized that special heat treatments coupled with these ranges of proportions will enhance these properties even further.

For several years air melted nickel base alloys containing about 2.5% titanium and about 1% aluminum were considered to possess the near optimum balance of high temperature strength consistent with reasonable forgeability. It was thought that larger additions of titanium and aluminum might increase the strengths but would surely decrease the ease of melting in air and forgeability to a non-commercial level. The entrance of vacuum melting into this field made possible an increase in the percentages of the reactive elements, better forgeability and improved properties.

Consequently, it is a primary object of our invention to produce improved nickel base alloys having a critical range of titanium and aluminum to produce for both low and high temperatures, high strength properties heretofore unpredictable and unexpected in reported wider alloy ranges.

Another object is to provide a nickel base alloy which, when made into sheet form, has unusual strength properties for both high and low temperature applications for lightweight design.

Still another object to provide a nickelbase alloy which when made into forgings, has improved strength properties especially in large discs.

An additional object is to provide heat treatment cycles which will enhance the increased high strength properties resulting from the use of a critical range of titanium and aluminum.

These and other objects of our invention will become apparent from the attached drawing, the detailed description and the claims which follow.

Briefly stated, in accordance with one aspect of our invention, we provide a composition range for an im-

2

proved nickel base alloy for use up to about 1800° F. comprising in percent by weight about 0.06-0.20 carbon, 18-20 chromium, 9-12 cobalt, 9-10.7 molybdenum, 3.0-3.3 titanium, 1.3-1.9 aluminum, up to about 0.02 boron, with the balance essentially nickel and impurities. In order to enhance our greater strength properties, we provide methods for heat treating our alloys to produce high tensile strength up to elevated temperatures comprising heating at about 1950° F. for about one-half hour, rapidly cooling to about room temperature and then heating at about 1400° F. for about 16 hours before cooling. In addition we provide methods for heat treating our alloys to produce high stress rupture strength up to elevated temperatures comprising, heating at about 2150° F. for about one half hour, rapidly cooling to about room temperature and then heating at a temperature of about 1650° F. for about four hours before cooling.

In studying various additions of aluminum and titanium to nickel base alloys containing molybdenum, we have noticed that very small changes in composition resulted in wide, unpredictable changes in properties. In addition, the combination of such new alloys with various heat treatments gave even higher, unexpected strength properties. Although such high strengths are attractive for 20 forgings, they are especially desirable and heretofore unavailable in sheet materials to be used at elevated temperatures, for example up to about 1800° F. In developing heat treatments and our critical composition range, it was necessary to prevent during cooling from 1950- 25 2150° F. the massive and untimely formation of undesirable phases of age hardening constituents which decrease the formability of high temperature aluminum-bearing, nickel base sheet alloys after heat treatment. Our improved alloy is essentially a new product since it has 30 properties which far exceed all reported sheet materials at elevated temperatures. Therefore its utility extends to temperatures higher than that of other known sheet 35 materials.

Two of the tests generally performed on alloys to discover their physical properties are "stress rupture" and "tensile" tests. The results of these tests, reported as "stress rupture strength" and "tensile strength" respectively, are generally defined as follows:

48 "Stress rupture strength" is the steady stress which a specimen will sustain without fracture for a given length of time (often 100 or 1000 hours).

"Tensile strength," sometimes called "ultimate strength," is the maximum stress which a specimen is capable of sustaining without fracture when the stress is continuously and quite rapidly increased during the testing period.

Both stresses mentioned above are obtained by dividing the load on the specimen at the time of fracture by the original cross sectional area of the untested specimen.

55 Our alloy when vacuum melted has the advantage of a 40% increase in tensile strength properties and a 60% increase in stress rupture strength over vacuum melted alloy A in Table I below and is 65% greater in tensile

strength and 50% greater in stress rupture strength than 60 vacuum melted alloy B in Table I below. Both alloys A and B are widely used high temperature materials. In addition, our alloy has remarkable formability and weldability properties despite the increase in titanium and aluminum over former usable similar alloys.

65 Our alloy range and its heat treatment will be better understood from our description taken in conjunction with the accompanying drawing and the following examples which are given by way of illustration only and not in any way by limitation. The scope of our invention will be pointed out in the claims.

In the drawings, Figure 1 is a graph the curves of which

compare stress rupture strength of our alloy with other currently available elevated temperature alloys.

Figure 2 is a graph the curves of which show the scatter band of stress rupture strength of sheet materials made from our broad alloy range.

As shown in Figures 1 and 2, stress rupture strengths are represented by a comparison of stress with a time-temperature parameter shown at the horizontal coordinate. This parameter has been calculated from the formula  $P = T(20 + \log t) \times 10^{-3}$  in which  $P$  = the time-temperature parameter number,  $T$  = absolute temperature in degrees Rankine and  $t$  = the time in hours.

These curves have been prepared from a large amount of stress rupture test results and represent a compact summary of such data. The nominal composition of alloys A, B, C, D and E of Figure 1 are compared in the following Table I:

Table I

## NOMINAL PERCENT BY WEIGHT

|            | Our Alloy | A       | B       | C       | D       | E       |
|------------|-----------|---------|---------|---------|---------|---------|
| Carbon     | 0.1       | 0.05    | 0.1     | 0.1     | 0.04    | 0.1     |
| Chromium   | 19        | 15      | 20      | 19      | 16      | 19      |
| Nickel     | balance   | 26      | 10      | balance | balance | balance |
| Iron       | balance   | balance | 3       | 4       | 10      | balance |
| Molybdenum | 10        | 1.3     | —       | 4       | —       | —       |
| Aluminum   | 1.7       | 0.2     | —       | 2.9     | 3.0     | 2.5     |
| Titanium   | 3.1       | 2.0     | —       | 2.9     | —       | .75     |
| Vanadium   | —         | 0.3     | —       | —       | —       | —       |
| Tungsten   | —         | —       | 15      | —       | —       | —       |
| Cobalt     | 11        | —       | balance | 19.5    | —       | 10      |

Figure 1 shows our alloy to be superior in stress rupture strength to currently available elevated temperature materials, the compositions of which are shown in Table I above, when all materials have been heat treated to give optimum stress rupture properties. The three strongest alloys of Figure 1, namely our alloy and alloys C and E, were solution heat treated in the 2000-2150° F. range. Although the composition of our alloy and of alloys C and E differ essentially only in the aluminum and titanium content, our alloy after being solution heat treated in the same range as alloys C and E, shows a marked increase in strength.

Figure 2 shows the upper and lower stress rupture ranges of our alloy when made into a series of sheet materials solution heat treated at 2150° F. for one hour and subsequently age hardened at 1650° F. for 4 hours from the following composition range in percent by weight: 0.06-0.20 carbon, 18-20 chromium, 9-12 cobalt, 9-10.7 molybdenum, 3.0-3.3 titanium, 1.3-1.9 aluminum, up to about 0.02 boron, up to about 0.5 silicon, up to about 0.5 manganese, up to about 5. iron with the balance essentially nickel.

## EXAMPLES 1-6

In order to determine initially the effect of aluminum on our alloy range, a series of alloys having the following compositions was vacuum melted:

Table II

| Example | Alloy | Elements (Percent by Wt.) |      |      |      |    |    |                |
|---------|-------|---------------------------|------|------|------|----|----|----------------|
|         |       | C                         | Al   | Ti   | Mo   | Cr | Co | Ni+Im-durities |
| 1       | E     | 0.1                       | 0.75 | 2.50 | 10.0 | 19 | 10 | Balance.       |
| 2       | J-40  | 0.1                       | 1.18 | 3.26 | 10.2 | 20 | 10 | Do.            |
| 3       | J-41  | 0.1                       | 1.60 | 3.27 | 10.7 | 20 | 10 | Do.            |
| 4       | J-42  | 0.1                       | 2.16 | 3.23 | 10.6 | 19 | 10 | Do.            |
| 5       | J-43  | 0.1                       | 2.75 | 3.22 | 10.6 | 20 | 10 | Do.            |
| 6       | J-44  | 0.1                       | 3.08 | 3.19 | 10.7 | 20 | 10 | Do.            |

The alloys of Examples 1-6 were then forged without difficulty into  $\frac{1}{2}$ " diameter bar stock. It is to be noted that the only alloy within our novel and critical range is that of Example 3. The alloys of Examples 1 and 2 contain lower percentages of aluminum, Example 1 having

a lower titanium content as well. Examples 4, 5 and 6 include aluminum at higher percentage ranges than our critical range. This bar stock was prepared for stress rupture testing by a solution heat treatment of about one hour at about 2100° F. in order to attain full solutioning and still obviate grain coarsening in the lower titanium and aluminum alloys. "Solution heat treatment" is a process in which an alloy is heated to a suitable temperature, is held at this temperature long enough to allow a certain constituent to enter into a solution called a solid solution and is then cooled rapidly to hold the constituent in solution. The metal is left in a supersaturated, unstable state and may subsequently exhibit "age hardening." The process of "age hardening" is a hardening process which by holding an alloy at a given temperature for a period of time increases hardness and strength.

All specimens were machined in this condition to proper testing configurations and subsequently age hardened at 1650° F. for about 20 hours. After age hardening, the reduced sections were hand polished to remove the small amount of oxide which had formed. Table III below compares the stress rupture strength of the alloys of Examples 1-6:

Table III

| Example | Alloy | 100 hour stress rupture strength (1,000 p.s.i.) |           |           |
|---------|-------|-------------------------------------------------|-----------|-----------|
|         |       | 1,500° F.                                       | 1,600° F. | 1,700° F. |
| 1       | E     | 32                                              | 18.5      | 14        |
| 2       | J-40  | 38.5                                            | 28        | 17.5      |
| 3       | J-41  | 40                                              | 30        | 19        |
| 4       | J-42  | 34.5                                            | 24.5      | 15.5      |
| 5       | J-43  | 35                                              | 24.5      | 16        |
| 6       | J-44  | 38.5                                            | 28        | 18.5      |

As seen in Table III, the alloy of Example 3 has higher stress rupture strength than any of the other alloys of Examples 1-6 thus showing a critical range and a peak of strength between 1.18% and 2.16% by weight aluminum.

In one of the tensile ductility tests which we made and which is a measure of the permanent deformation before fracture by stress in tension, we compared one alloy including a lower percentage of aluminum and one alloy including a higher percentage of aluminum with an alloy within our novel range. The following Table IV which shows a tensile ductility comparison at 1500° F. reports ductility as percent elongation, the amount of permanent extension in the fracture area in a tension test, and also as percent reduction in cross sectional area that occurred during the stress application.

Table IV

| Example Alloy | Percent Elongation (in 1 inch) | Percent Reduction in Area |
|---------------|--------------------------------|---------------------------|
| 2             | 19                             | 59                        |
| 3             | 31                             | 60                        |
| 5             | 26                             | 57                        |

It is to be noted that in addition to having a higher stress rupture strength than the other alloys of this series, our alloy of Example 3 also has the best tensile ductility.

### EXAMPLES 7-9

Although we had obtained excellent results using bar stock made from material within our critical alloy range, we were extremely interested in producing from our alloy a sheet material which would have superior properties. A problem existing in the production of sheet materials from aluminum-bearing, nickel base alloys is the prevention upon cooling after heat treatment of the massive formation of undesirable phases of age hardening constituents which decrease the formability of such sheet material.

The following Examples 7-9 show the results of our heat treating an alloy within our critical composition range to overcome the formation of undesirable phases in our alloy sheet. For use in Examples 7-9 an alloy heat No. 3-985 of the following composition within our novel range was melted and formed into sheet material of 0.063" thickness:

#### Percent by weight

|                       |         |
|-----------------------|---------|
| Carbon                | 0.15    |
| Aluminum              | 1.7     |
| Titanium              | 3.1     |
| Molybdenum            | 10.5    |
| Chromium              | 19.1    |
| Cobalt                | 9.4     |
| Silicon               | 0.03    |
| Manganese             | 0.03    |
| Nickel and impurities | Balance |

We used the following heat treatment cycles:

*Example 7.*—Solution heat treat at 1950° F. for one-half hour, air cool to about room temperature, age harden at 1400° F. for sixteen hours and then air cool.

*Example 8.*—Solution heat treat at 2150° F. for one-half hour, air cool to about room temperature, age harden at 1400° F. for sixteen hours and then air cool.

*Example 9.*—Solution heat treat at 2150° F. for one-half hour, air cool to about room temperature, age harden at 1650° F. for sixteen hours and then air cool.

Table V below compares stress rupture data obtained from sheet material heat treated according to Examples 7 and 9.

Table V

| Temperature<br>(° F.) | Stress<br>(1,000 p.s.i.) | Hours-to-Failure After<br>Heat Treatment |           |
|-----------------------|--------------------------|------------------------------------------|-----------|
|                       |                          | Example 7                                | Example 9 |
| 1,600                 | 35                       | 94                                       | 150       |
| 1,650                 | 20                       | 47                                       | 112       |
| 1,800                 | 10                       | 69                                       | 141       |

A series of specimens were prepared from the 0.063" thick sheet material obtained from our alloy heat No. 3-985 by heat treating according to Examples 7 and 8. These specimens were then shaped into the proper form for tensile strength testing. In addition to the tensile strength, we determined the 0.2% yield strength which is the stress at which a material exhibits 0.2% permanent extension. This figure, sometimes called "0.2% offset," is commonly used as a design criterion for strength.

The following Table VI shows the variation of tensile

strength properties of our alloys with heat treatment cycles:

Table VI

| Temperature (° F.) | Tensile Strength<br>(1,000 p.s.i.) |                    | 0.2% Yield Strength<br>(1,000 p.s.i.) |                    |
|--------------------|------------------------------------|--------------------|---------------------------------------|--------------------|
|                    | H. T.<br>Example 7                 | H. T.<br>Example 8 | H. T.<br>Example 7                    | H. T.<br>Example 8 |
| Room               | 191.5                              | 152                | 150                                   | 123                |
| 1,200              | 107                                | 105                | 135                                   | 108.5              |
| 1,300              | 167                                | 105                | 127.5                                 | 98.5               |
| 1,400              | 137                                | 115                | 119.5                                 | 102.5              |
| 1,500              | 115.5                              | 107                | 107.5                                 | 93                 |

As seen from Table VI above, the heat treatment of Example 7 results in superior properties to that of Example 8. Comparing the results of both stress rupture and tensile strength variations with heat treatments, it is noted that to obtain superior stress rupture strength, it is better to solution heat treat at 2150° F. rather than at 1950° F. and to age harden at 1650° F. rather than 1400° F.; and in order to obtain superior tensile strength, it is better to solution heat treat at 1950° F. rather than at 2150° F. and to age harden at 1400° F. These unusual characteristics for our alloy allow us to designate a different heat treatment in order to obtain either high stress rupture strength or high tensile strength, whichever the designer of an article may require.

### EXAMPLE 10

In order to compare our alloy heat treated to its optimum strength with an alloy whose composition closely resembles that of our alloy but was slightly different in the titanium and aluminum content, we prepared sheet materials from the following two alloys:

| Alloy | Percent by Weight |      |     |     |      |     |                    |
|-------|-------------------|------|-----|-----|------|-----|--------------------|
|       | C                 | Al   | Ti  | Mo  | Cr   | Co  | Ni +<br>Impurities |
| M-252 | 0.19              | 1.15 | 2.5 | 9.7 | 20.0 | 9.9 | Balance            |
| J-41A | 0.15              | 1.66 | 3.1 | 9.4 | 19.1 | 9.4 | Do                 |

The results of tensile testing on sheet material prepared from these alloys and heat treated according to the optimum conditions given in Example 7 are shown in the following Table VII:

Table VII

| Temp. (° F.) | Tensile Strength<br>(1,000 p.s.i.) |       | 0.2% Yield Strength<br>(1,000 p.s.i.) |       |
|--------------|------------------------------------|-------|---------------------------------------|-------|
|              | M-252                              | J-41A | M-252                                 | J-41A |
| Room         | 180                                | 183   | 79                                    | 118   |
| 1,000        | 157                                | 166   | 71                                    | 103   |
| 1,200        | 152                                | 162   | 70                                    | 100   |
| 1,400        | 119                                | 133   | 66                                    | 87    |
| 1,600        | 70                                 | 91    | 36                                    | 56    |

From Table VII it is easily apparent that the small variation in titanium and aluminum content, coupled with an optimum heat treatment gives a greatly improved tensile strength results.

A test used for determining the formability of an alloy is known as the "Erichsen Cup Test." It is a type of ductility test for sheet material which measures the depth in millimeters of an impression at fracture, made by forcing a cone-shaped plunger into a specimen. The greater the depth of depression, the better is the formability. The following Table VIII shows the results of Erichsen Cup testing on the alloys of this example which were solution heat treated at 1950° F. for one half hour and then cooled as indicated. Although the compositions of M-252 and our J-41A are essentially the same except

for the critical variation in aluminum and titanium content, our J-41A has a much higher degree of formability.

Table VIII

| Alloy   | Rapid Cooling       |                           |
|---------|---------------------|---------------------------|
|         | Depth of Draw (in.) | Max. Force (1,000 p.s.i.) |
| J-41A   | .424                | 16.2                      |
|         | .451                | 17.6                      |
|         | .447                | 17.8                      |
|         | .446                | 17.6                      |
|         | .330                | 16.2                      |
|         | .339                | 16.9                      |
| M-252-A | .341                | 17.4                      |
|         | .345                | 16.8                      |

## EXAMPLES 11-12

Although without boron our alloy has properties superior to other alloys, certain physical characteristics are improved by the inclusion of boron. To exemplify these increased properties, we melted alloys of the following compositions:

| Example | Heat No. | Percent by Weight |      |    |    |      |      |       |                   |
|---------|----------|-------------------|------|----|----|------|------|-------|-------------------|
|         |          | C                 | Cr   | Co | Mo | Ti   | Al   | B     | Ni and Impurities |
| 11      | VA-157   | .1                | 18.6 | 11 | 10 | 3.12 | 1.78 | 1.003 | Balance. Do.      |
| 12      | V-5      | .1                | 18.7 | 10 | 10 | 3.17 | 1.89 | .005  | Balance. Do.      |

1 Max.

Table IX below compares the stress rupture strengths of the alloys of Examples 11 and 12 and shows that an increase in boron increases strength. The alloys of Examples 11 and 12 were each solution heat treated at 2150° F. for about one half hour, air cooled to about room temperature, age hardened at about 1650° F. for about 4 hours and then cooled.

Table IX

| Example | Temperature (° F.) | Stress (1,000 p.s.i.) | Hours to Failure |
|---------|--------------------|-----------------------|------------------|
| 11      | 1,200              | 110                   | 72.5             |
| 12      | 1,200              | 110                   | 152.1            |
| 11      | 1,500              | 50                    | 14.4             |
| 12      | 1,500              | 50                    | 36.5             |
| 11      | 1,650              | 25                    | 25.1             |
| 12      | 1,650              | 25                    | 53.9             |
| 11      | 1,800              | 10                    | 31.0             |
| 12      | 1,800              | 10                    | 97.5             |

## EXAMPLE 13

One way of representing the relationship of stress rupture strength to time and temperature is to use the formula  $P = T(20 + \log t) \times 10^{-3}$  as defined before. Some data from which the scatter band of Figure 2 was produced and data which is representative of our alloy range when solution heat treated at about 2150° F. for one half hour, air cooled to about room temperature, age hardened at about 1650° F. for about 4 hours and then air cooled is given in Table X:

Table X

| Temperature (° F.) | Stress (p.s.i.) | Hours to Failure |       |       | Parameter |      |      |
|--------------------|-----------------|------------------|-------|-------|-----------|------|------|
|                    |                 | Min.             | Avg.  | Max.  | Min.      | Avg. | Max. |
| 1,200              | 110,000         | 16               | 80    | 160   | 35.2      | 36.3 | 36.8 |
| 1,200              | 95,000          | 100              | 450   | 634   | 36.5      | 37.5 | 37.8 |
| 1,350              | 70,000          | 32               | 100   | 160   | 38.8      | 39.8 | 40.1 |
| 1,350              | 55,000          | 400              | 1,000 | 1,590 | 40.8      | 41.5 | 41.9 |
| 1,400              | 40,000          | 1,000            | 1,410 | 2,520 | 42.7      | 43.0 | 43.5 |
| 1,500              | 33,000          | 250              | 316   | 634   | 43.8      | 44.0 | 44.6 |
| 1,650              | 20,000          | 63               | 160   | 225   | 46.0      | 46.4 | 47.2 |
| 1,800              | 10,000          | 22               | 80    | 159   | 48.1      | 49.4 | 50.0 |

An additional example of the average tensile strength of our alloy is given in Table XI below. This data was accumulated from tensile tests of sheet material solution heat treated at 1950° F. for one half hour, air cooled to room temperature, age hardened at 1400° F. for sixteen hours and then air cooled.

Table XI

| Temperature (° F.) | Avg. Ultimate Strength (1,000 p.s.i.) | Avg. 0.2% Yield Strength (1,000 p.s.i.) | Avg. Percent Elongation (inches/inch) |
|--------------------|---------------------------------------|-----------------------------------------|---------------------------------------|
| 10                 |                                       |                                         |                                       |
| 15 Room Temp.      | 143                                   | 102                                     | 11.5                                  |
| 1200               | 138                                   | 92                                      | 15                                    |
| 1300               | 132                                   | 95                                      | 12                                    |
| 1400               | 127                                   | 97                                      | 8.5                                   |
| 1500               | 102                                   | 81                                      | 8.3                                   |
| 1650               | 65                                    | 66                                      | 8.0                                   |
| 1800               | 39                                    | 33                                      | 13.5                                  |

In the foregoing description we have disclosed an

improved nickel base alloy for use up to about 1800° F. and methods of heat treatment for such alloy to enhance the improved strength properties depending on intended use. Although we have described our invention in connection with specific examples, these examples are to be construed as illustrative of rather than limitations on our invention. Those skilled in the art of metallurgy and heat treatment will readily understand the modifications and variations of which our invention is capable, for example, as to the limit of allowable variation of time, temperature and atmosphere in heat treatment cycles and as to the variation of the composition of our alloy within the limits of alloy melting procedures and quantitative analytical methods. We intend in the appended claims to cover modifications and variations that come within the true spirit and scope of our invention.

What we claim as new and desire to secure by Letters Patent of the United States is:

1. An improved nickel base alloy suitable for use at elevated temperatures comprising in percent by weight: 0.06-0.20 carbon; 18-20 chromium; 9-12 cobalt; 9-10.7 molybdenum; 3.0-3.3 titanium; 1.3-1.9 aluminum; with the balance essentially nickel and impurities.

2. The alloy of claim 1 which includes up to about 0.02% by weight boron.

3. The alloy of claim 1 which includes in percent by weight: up to 0.5 silicon; up to 0.5 manganese; and up to 5. iron.

4. An improved nickel base alloy suitable for use at elevated temperatures comprising in percent by weight: 0.06-0.12 carbon; 18-20 chromium; 10-12 cobalt; 9-10.7 molybdenum; 3.0-3.3 titanium; 1.3-1.8 aluminum; up to about 0.02 boron; with the balance essentially nickel and impurities.

5. An improved nickel base alloy suitable for use at elevated temperatures comprising in percent by weight: 0.06-0.12 carbon; 18-20 chromium; 10-12 cobalt; 9-10.7 molybdenum; 3.0-3.3 titanium; 1.3-1.8 aluminum; 0.0005-0.015 boron; with the balance essentially nickel and impurities.

6. An improved nickel base alloy suitable for use at elevated temperatures comprising in percent by weight: 0.08-0.15 carbon; 18.5-19.5 chromium; 9.4-11 cobalt; 9.3-10.7 molybdenum; 3.0-3.2 titanium; 1.3-1.9 aluminum; 0.001-0.010 boron; with the balance essentially nickel and impurities. 5

## References Cited in the file of this patent

## UNITED STATES PATENTS

|           |                   |              |
|-----------|-------------------|--------------|
| 2,712,498 | Gresham et al.    | July 5, 1955 |
| 2,747,993 | Johnson           | May 29, 1956 |
| 2,766,155 | Betteridge et al. | Oct. 9, 1956 |